

# UNITED STATES PATENT OFFICE.

WILLIAM ROY MOTT, OF LAKEWOOD, OHIO, ASSIGNOR TO NATIONAL CARBON COMPANY, INC., A CORPORATION OF NEW YORK.

## ARC-LAMP ELECTRODE.

1,311,133.

Specification of Letters Patent.

Patented July 22, 1919.

No Drawing.

Application filed October 2, 1918. Serial No. 256,600.

To all whom it may concern:

Be it known that I, WILLIAM R. MOTT, a citizen of the United States, residing at Lakewood, in the county of Cuyahoga and State of Ohio, have invented a certain new and useful Improvement in Arc-Lamp Electrodes, of which the following is a full, clear, and exact description.

This invention relates particularly to improvements in arc lamp electrodes although the phenomena disclosed may be utilized in electrodes for other purposes.

The object of the invention is to obtain an artificial source of light of high intrinsic 15 brilliancy and increased candle power.

Another object of the invention is to secure an intensely brilliant source of light approximating a point source which is the ideal illumination for projector arc lamps and 20 searchlights.

The positive crater of the carbon arc has always been supposed to have the highest intrinsic brilliancy of any source of light, and is also the nearest approximation to a 25 point source of light of high candle power. The highest temperatures readily obtainable heretofore for various investigations also are found in the positive crater of the carbon arc.

30 I have found new means by which it is possible to secure an intensely bright positive crater which is of much greater brilliancy than the carbon arc and also has a higher arc temperature.

35 The materials which have been found to produce this result are metallic tantalum and certain tantalum compounds, particularly the oxid and carbide. These materials are preferably embodied either alone or 40 combined with other flaming materials, in the core of a positive carbon electrode, or as a wire in the center of the electrode. The combination of tantalum and zirconium is especially good. A carbon shell containing 45 about 50% of zirconium oxid gave the most steady arc. The cross section of the core or the diameter of the wire may be varied depending on the result desired, but the sizes are preferably about the same as those 50 of the ordinary open arc flame cored carbons. The negative is preferably carbon although an electrode containing flaming material may be used. It has previously been believed and reported in the literature

that all flaming materials decrease the arc 55 and crater temperatures of the carbon arc, but I have found that tantalum increases the arc temperature and is a marked exception to this rule. On burning an electrode having tantalum incorporated therein, this 60 phenomena is evidenced by the unique fact that the carbon is pitted at the points where the arc strikes the tantalum, very probably because the tantalum has been raised to such a high temperature that the carbon below 65 it has been volatilized. The arc stream is very concentrated at the point where the arc rests on the tantalum and the candle power of the arc as a whole is considerably increased by the very small intensely brilliant 70 crater.

A current of at least 6 amperes, and preferably 20 to 50 amperes, is desirable to best develop the small, very bright, white incandescent positive crater. The light is whiter 75 than that obtained in lower temperature carbon arcs, principally because the temperature is higher.

In investigations with the arc spectrum, the increased temperature attainable may be 80 a means of decidedly modifying the spectrum previously obtained with the carbon arc.

Having described my invention, what I claim is:

1. An electrode containing carbon and tantalum.
2. A positive electrode containing carbon and tantalum material.
3. An electrode containing carbon and 85 having a core containing a tantalum material.
4. A positive electrode containing carbon and a core of metallic tantalum.
5. In arc lamps, the combination of a 90 positive electrode containing tantalum and a negative electrode containing carbon.
6. An electrode containing carbon, tantalum and zirconium.
7. A positive electrode containing carbon 100 and zirconium and having a core containing tantalum.
8. A positive electrode containing carbon and zirconium oxid and having a core containing a tantalum material.

In testimony whereof, I hereunto affix my signature.

WM. ROY MOTT.